

## UNITED STATES PATENT OFFICE

2,612,469

RAPID FINE-GRAINED COPPER  
ELECTRODEPOSITION

Frederick F. Reisinger, Willoughby, Ohio, assignor to The Wire Coating and Manufacturing Company, Cleveland, Ohio, a corporation of Ohio

No Drawing. Application September 28, 1948.  
Serial No. 51,639

7 Claims. (Cl. 204—52)

**1** Copper plating by means of copper cyanide is quite an old industry, and from time to time detailed improvements in bath compositions have been suggested, such as the Rochelle salt copper bath, pyrophosphate copper, etc., but a fundamental handicap has remained that plating could not be operated at high current densities as desirable for volume production. Even plating with as low as 12-15 amperes per sq. ft. has resulted in deposits more or less rough and pitted if a thickness 0.001" or more was required. A bath for electrodeposition which can permit high operating rates, with current densities of 30 or more amperes per sq. ft., and with production of bright fine-grained deposits has accordingly been much desired in the industry. In accordance with the present invention, an improved electrodeposition thus with high current density and volume production of smooth fine-grained bright deposits in such thicknesses as may be desired, is now possible. Other objects and advantages of the invention will appear in the following description.

To the accomplishment of the foregoing and related ends, the invention then comprises the features hereinafter fully described, and particularly pointed out in the claims, the following description setting forth in detail certain illustrative embodiments of the invention, these being indicative however of but a few of the various ways in which the principle of the invention may be employed.

In general, copper is supplied by a bath of copper cyanide type, and of alkaline category. Fundamentally, in the present invention the bath is provided with a reaction product of a diazo salt and sulphur, such product being dissolved and made up with the desired copper cyanide and other ingredients for the operating bath.

For the preparation of the diazo derivative, the starting point is a primary arylamine, preferably anthranilic acid, but there may be also applied aniline and its homologs, the toluidines and xylydines, also benzylamine, etc. Thus for instance the anthranilic acid or other arylamine is made up in an acid solution, for instance hydrochloric, although sulphuric or other equivalent mineral acids may be used, then sodium nitrite or equivalent diazotizing agent in solution is applied. The diazo salt as thus provided in solution is reacted with sulphur in a precipitating form, such as hydrogen sulphide, sodium sulphide, etc. Conveniently, hydrogen sulphide is passed into the solution for around two hours,

or as necessary to complete precipitation. The resulting precipitate which may be designated a "reaction product of a sulphide on a diazo salt of a primary arylamine," is vacuum-filtered as dry as possible, and the filter cake is dissolved and with further advantage is boiled in water containing triethanolamine. After cooling and filtering, the filtrate is mixed with a solution of copper cyanide, sodium cyanide and sodium hydroxide, and is boiled, cooled and filtered, a wetting agent, such for instance as a sulphate of a long chain alcohol, preferably of 10-14 carbon atoms, diethyl sodium sulphosuccinate, alkaryl sodium sulphonates, etc. is added, and desirably the final volume is made up with addition of water as necessary, to a convenient concentration stock solution. A desired amount of this concentration is added to the cyanide copper bath which is to be operated.

**20** With such bath, high current density is employed, conveniently 30-50 amperes per sq. ft. The copper deposited is smooth, fine-grained, and bright, and thickness of 0.001" can thus be readily obtained in about 15 minutes.

**25** For example: 1.08 kg. of anthranilic acid is dissolved in 1.62 liters of water and 1.19 of concentrated hydrochloric acid. Then 810 gms. of sodium nitrite in 7.6 liters of water is added.

After the diazotizing action is completed, a stream of hydrogen sulphide is passed through the solution for about two hours. The resulting precipitate is filtered and vacuum sucked dry as much as possible. This sulphide-precipitated diazo compound provides the active agent in my high-speed plating bath. The filter cake is then dissolved and boiled for about 30 minutes in a solution of 5.8 liters of triethanolamine in 29 liters of water. The solution is cooled and filtered. The filtrate is mixed with 10.16 liters of a solution of the following composition: 392 gms. of copper cyanide and 438 gms. of sodium cyanide and 99 gms. of sodium hydroxide per gallon or 3.785 liters. This mixture is brought to a boil, then cooled and filtered. And to the filtrate 210 cc. of a sulphate of long chain alcohol wetting agent is added and the final volume is made up to 24 gallons or 90.84 liters. This stock solution is then employed by adding to the copper cyanide bath for operation. For instance, 50 to 75 cc. of the stock solution is added for each gallon of any copper cyanide electrodeposition bath.

Other modes of applying the principle of the invention may be employed, change being made as regards the details described, provided the

features stated in any of the following claims, or the equivalent of such, be employed.

I therefore particularly point out and distinctly claim as my invention:

1. In a process of preparing a bath for electrodepositing copper, dissolving anthranilic acid in hydrochloric acid solution, reacting upon the same with a diazotizing agent, then precipitating by  $H_2S$ , de-watering the precipitate, dissolving the precipitate and boiling in triethanolamine and water, cooling, filtering, mixing with a solution containing copper cyanide, sodium cyanide and sodium hydroxide, boiling, cooling, filtering, adding a wetting agent, making to a stock volume with water, and adding a minor proportion of such stock solution to an electrodeposition bath containing copper cyanide, sodium cyanide and sodium hydroxide.

2. In a process of preparing a bath for electrodepositing copper, forming a diazo salt of a primary arylamine of the group consisting of anthranilic acid, aniline, toluidines, xylidines and benzylamine, in a mineral acid solution, precipitating by hydrogen sulphide, de-watering the precipitate, dissolving the precipitate and boiling in triethanolamine and water, cooling, filtering, mixing with a solution containing copper cyanide, sodium cyanide and sodium hydroxide, boiling, cooling, filtering, adding a wetting agent, making to a stock volume with water, and adding a minor proportion of such stock solution to an electrodeposition bath containing copper cyanide, sodium cyanide and sodium hydroxide.

3. In a process of preparing a bath for electrodepositing copper, forming a precipitate by reacting on a solution of diazo salt of a primary arylamine of the group consisting of anthranilic acid, aniline, toluidines, xylidines and benzylamine, with a sulphide precipitant of the group consisting of hydrogen sulphide and sodium sulphide, de-watering the precipitate, dissolving the precipitate and boiling in triethanolamine and water, filtering and mixing with a solution containing copper cyanide and sodium cyanide and sodium hydroxide, boiling, filtering, adding a wetting agent, making up to a stock volume solution with water, and adding a minor proportion of such stock solution to a copper cyanide electrodeposition bath.

4. In a process of preparing a bath for electrodepositing copper, forming a precipitate by reacting on a solution of diazo salt of a primary

arylamine of the group consisting of anthranilic acid, aniline, toluidines, xylidines and benzylamine, by a sulphide precipitant of the group consisting of hydrogen sulphide and sodium sulphide, de-watering the precipitate, dissolving the precipitate in water containing triethanolamine, and supplying such solution to a copper cyanide electrodeposition bath.

5. In a process of the character described, electrodepositing copper from a solution which contains copper cyanide, sodium hydroxide, and a reaction product of a sulphide of the group consisting of hydrogen sulphide and sodium sulphide on a diazotized primary arylamine of the group consisting of anthranilic acid, aniline, toluidines, xylidines and benzylamine, said reaction product as a precipitate being dissolved in water containing triethanolamine.

6. A plating bath of aqueous copper cyanide and sodium hydroxide, including the reaction product of a sulphide of the group consisting of hydrogen sulphide and sodium sulphide on diazotized anthranilic acid, said reaction product as a precipitate being dissolved in water containing triethanolamine.

7. An electrodeposition bath including copper cyanide, sodium hydroxide, and the reaction product of a sulphide of the group consisting of hydrogen sulphide and sodium sulphide on a diazotized primary arylamine of the group consisting of anthranilic acid, aniline, toluidines, xylidines, and benzylamine, said reaction product as a precipitate being dissolved in water containing triethanolamine.

35 FREDERICK F. REISINGER.

#### REFERENCES CITED

The following references are of record in the file of this patent:

#### 40 UNITED STATES PATENTS

| Number       | Name            | Date          |
|--------------|-----------------|---------------|
| 2,195,409    | Flett           | Apr. 2, 1940  |
| 2,271,209    | Schlotter       | Jan. 27, 1942 |
| 45 2,287,654 | Wernlund et al. | June 23, 1942 |
| 2,424,887    | Henricks        | July 29, 1947 |
| 2,471,918    | Willson et al.  | May 31, 1949  |
| 2,495,668    | Willson et al.  | Jan. 24, 1950 |

#### FOREIGN PATENTS

| Number  | Country       | Date          |
|---------|---------------|---------------|
| 199,706 | Great Britain | Feb. 14, 1924 |